

# UNITED STATES PATENT OFFICE.

TITO RONDELLI, OF TURIN, AND QUIRINO SESTINI, OF BERGAMO, ITALY, ASSIGNEES  
OF ONE-THIRD TO SESTRON (FOREIGN PATENTS) LIMITED, OF LONDON, ENGLAND.

## COLORATION OF METALLIC SURFACES.

1,417,413.

Specification of Letters Patent. Patented May 23, 1922.

No Drawing.

Application filed June 30, 1920. Serial No. 393,198.

To all whom it may concern:

Be it known that we, TITO RONDELLI and QUIRINO SESTINI, subjects of the King of Italy, residing at Turin, Italy, and Bergamo, Italy, respectively, have invented certain new and useful Improvements in the Coloration of Metallic Surfaces, (for which on October 27, 1916, we filed an application No. 156,509 for Letters Patent of Italy), of which the following is a specification.

This invention relates to the coloration of metallic surfaces, and has for its object to provide an improved process for this purpose.

In the prior British specification, No. 106774 (No. 16582/16) a process for bronzing or colouring metallic surfaces is described according to which the surface to be bronzed or coloured is electrolytically coated with copper from an electrolyte which is a hot dense alkaline solution, (for example, having a temperature of about 120-140° C and a density about 1.3-1.5) containing an oxide of copper combined with the alkali, and the surface is then coloured or bronzed, for example, by anodic oxidation in the electrolytic bath. It has now been found that a modification of this process is specially adaptable for the coloration of metallic surfaces, such as copper and ferrous surfaces.

According to the present invention the improved process for colouring metallic surfaces consists in immersing the object, the surface of which is to be coloured, in a warm or hot electrolytic bath containing a fixed alkali in which is dissolved, preferably to saturation or substantially so, a compound of copper, for example, cupric oxide or hydrate, the object under treatment being made to serve exclusively as anode for a shorter or longer period.

The copper bath may be prepared in any suitable way by chemical or electro-chemical means, for example, by dissolving cupric oxide, or better, cupric hydrate, in a solution of caustic alkali, such as caustic soda. Instead of the oxide or hydrate any suitable copper compound which will be similarly and dissolve in the excess of alkali may be used, for example, copper sulphate. The concentration of the bath may vary within considerable limits, but

preferably is such that the solution boils at a comparatively high temperature, for example 120-150° C. A wide range of current density is applicable, for instance, from 1-30 amperes per square decimeter of the surface to be coloured, the particular density employed depending, of course, upon the circumstances of the case. For certain copper alloys it will be found that a comparatively low current density should be used, such as one from 3-5 amperes per square decimeter, while in other cases, as when the surface under treatment consists of substantially pure copper or of bronze of high copper content, a density of from 10-12 amperes may be conveniently employed. As will be readily understood, the conditions in any given case will be determined by the nature of the surface to be coloured as well as by the nature of the object and the particular effect desired. The same considerations apply to the temperature and to the time during which the object is immersed. When copper alloys are in question the concentration of the bath and the temperature depend in particular upon the constitution of the alloy. In every case, however, a simple preliminary experiment suffices to determine the most advantageous conditions necessary to obtain the result desired. By varying the conditions different effects, from light green and dark blue colours through darker colorations up to black, may be produced.

The following examples will serve to indicate the character of the invention in more detail, but it is to be understood that these examples are given as illustrative only and not by way of limitation.

### Example I.

Copper oxide is dissolved to saturation in a solution of caustic soda which boils between about 120-130°. The bath so prepared is maintained at a temperature of from 90-130° and a copper article, the surface of which has been previously cleaned, mechanically or otherwise, is immersed, being made the anode in the bath, and a current of a density of 12 amperes per square decimeter of the surface is passed for about 5 minutes. The surface is thereby extensively oxidized, coloured black, rendered re-

sistant to corrosive agencies and can be polished with excellent effect.

*Example II.*

5. A brass sheeting containing from 60-75% copper, 25-40% zinc and 1-3% lead, is made the anode in the same bath as in Example I, under current density of 5 amperes per square decimeter, the temperature being 75° 10 and the time of immersion about 2 minutes. A similar result is obtained as in the previous case. If the treatment be applied only for a few seconds iridescent effects are produced.

15

*Example III.*

An iron object is immersed in the same bath as in the previous examples, the temperature being between 90-130°, and is submitted to anodic oxidation under a current density not exceeding 5 amperes per square decimeter. After about 5-20 minutes treatment, according to the constitution of the iron, and the condition of the surface, the 20 latter is coloured a deep blue black.

Not infrequently, copper and copper alloy surfaces are coloured by deposition thereon of arsenic, or even, in some cases, of platinum, but coloration is more generally effected by treatment in solutions of alkali sulphides or sulphides of alkali earths, and it has also been the practice to employ a solution of copper nitrate, or of copper carbonate in ammonia. The three first processes, however, do not give satisfactory results either in respect to the colour produced, or to its permanence, while the last two methods are not easy of application, and regular effects are difficult to obtain. The 35 present invention provides a simple and expeditious means of colouring metallic surfaces, and of obtaining varied effects with facility and regularity.

A process for oxidizing ferrous surfaces 45 by treating the same without the use of an electric current in an alkaline bath containing the oxide of a metal which behaves electro-negatively towards iron is described and, claimed in our co-pending application Serial 50 No. 393,199, filed June 30, 1920.

What we claim as our invention and desire to secure by Letters Patent is:—

1. The process for colouring metallic surfaces which comprises submitting the surface to be coloured to anodic oxidation in the presence of a concentrated alkaline electrolyte containing copper.

2. The process for colouring metallic surfaces which comprises immersing the object 60 the surface of which is to be coloured in a concentrated solution of fixed alkali in which is dissolved a compound of copper and submitting the surface to anodic oxidation.

3. The process for colouring metallic surfaces which comprises immersing the object 65

the surface of which is to be coloured in a concentrated solution of fixed alkali in which is dissolved a compound of copper and submitting the surface to anodic oxidation with application of heat.

4. The process for colouring metallic surfaces which comprises immersing the object 70 the surface of which is to be coloured in a concentrated solution of fixed alkali in which is dissolved to saturation a compound of copper and submitting the surface to anodic oxidation.

5. The process for colouring metallic surfaces which comprises immersing the object 75 the surface of which is to be coloured in a solution of fixed alkali of a density of 1.3-1.5 in which is dissolved a compound of copper and submitting the surface to anodic oxidation.

6. The process for colouring metallic surfaces which comprises immersing the object 80 the surface of which is to be coloured in a solution of caustic alkali of a density of 1.3-1.5 in which is dissolved a compound of copper and submitting the surface to anodic oxidation.

7. The process for colouring metallic surfaces which comprises immersing the object 85 the surface of which is to be coloured in a solution of caustic soda of a density of 1.3-1.5 in which copper oxide is dissolved to saturation and submitting the surface to anodic oxidation.

8. The process for colouring metallic surfaces which comprises immersing the object 90 the surface of which is to be coloured in a solution of caustic soda of a density of 1.3-1.5 in which copper oxide is dissolved to saturation and submitting the surface to anodic oxidation with application of heat.

9. The process for colouring a copper surface which comprises immersing the object 95 the surface of which is to be coloured in a concentrated solution of fixed alkali in which is dissolved a compound of copper and submitting the surface to anodic oxidation.

10. The process for colouring a copper surface which comprises immersing the object 100 the surface of which is to be coloured in a solution of caustic soda, having a boiling-point between about 120°-130°, in which copper oxide is dissolved to saturation and submitting the surface to anodic oxidation with application of heat.

In testimony whereof we have signed our 120 names to this specification in the presence of two subscribing witnesses.

TITO RONDELLI.

QUIRINO SESTINI.

Witnesses to signature of Tito RONDELLI:

J. PHILLIPS CRAWLEY,

J. W. PATCHING.

Witnesses to signature of QUIRINO SESTINI:

DANTE DANIELH,

ANSELMO VILLY,